

E. J. SCHRODER,  
BUILDING MATERIAL.  
APPLICATION FILED JAN. 21, 1914.

1,218,217.

Patented Mar. 6, 1917.

FIG.1.



FIG.2.



Asbestos paper saturated with  
non-asphaltic waterproofing material.

FIG.3.



Witnesses:

J. C. Derrick.  
Verma Stuart

Inventor:

Edward J. Schroder  
By Miller & Chindahl  
Atty.

# UNITED STATES PATENT OFFICE.

EDWARD J. SCHRODER, OF CHICAGO, ILLINOIS.

## BUILDING MATERIAL.

1,218,217.

Specification of Letters Patent.

Patented Mar. 6, 1917.

Application filed January 21, 1914. Serial No. 813,394.

*To all whom it may concern:*

Be it known that I, EDWARD J. SCHRODER, a citizen of the United States, residing at Chicago, in the county of Cook and State 5 of Illinois, have invented certain new and useful Improvements in Building Material, of which the following is a specification.

Although asbestos paper is used to some extent as a surfacing for prepared roofing, 10 it is but poorly adapted to withstand the effects of the weather. Asbestos paper is very soft and absorbent, and when wet its fibers may be readily "scuffed" off, hence those fibers which are not held in place by 15 reason of adhesion to the asphalt contained in the roofing are loosened and removed by the elements in a comparatively short time.

One of the objects of this invention is to render asbestos paper waterproof and to 20 bind together the fibers thereof, thus adapting the paper to withstand the effects of exposure to the weather.

Another object is to accomplish the waterproofing of asbestos paper without the use 25 of asphalt or other dark-colored substances, in order that the surface of the paper shall present a light or approximately white ground capable of having colors and designs imprinted thereon.

It will be apparent that a sheet of asbestos paper treated as hereinbefore suggested is well adapted for use as the outer covering 30 of building material other than roofing, as, for example, wall-board and siding.

I have found that an oil, either oxidized 35 or capable of oxidation in contact with air, dissolved in a suitable solvent, constitutes a satisfactory material for waterproofing asbestos paper. The oil may be what is known as a prepared oil, or what is termed a drying oil, such as linseed oil, poppyseed oil, menhaden oil, tung oil (Chinese wood oil), etc. If desired, rubber or a rubber substitute may be used in combination with the 40 oil. The solvent may be naphtha, benzine or other suitable material.

After saturation in a waterproofing solution such as just described, asbestos paper acquires a waterproof, hard, wear-resisting 45 surface, and possesses a greater degree of rigidity than the untreated paper. The color of the treated paper is somewhat darker than that of the unwaterproofed paper, but is still sufficiently light to permit of colors or designs being applied thereto. If the sheet is to be given a solid

color, the coloring material may be mixed with the waterproofing solution, or it may be applied to the sheet after the latter has been waterproofed. If it is desired to place 50 upon the sheet a design simulating shingles, tiles, or slate, or any other arrangement of forms or colors (a few examples of which are indicated in Fig. 3), such design or arrangement may be imprinted upon the 55 sheet either before or after the sheet has been waterproofed.

When the asbestos sheet is to be used as the protective coating of prepared roofing, the waterproofing solution may, if desired, 60 be applied after the sheet has been united with the body of the roofing, but it is preferred to waterproof the asbestos sheet prior to application of the sheet to the roofing body.

The waterproofed asbestos paper constitutes an article of manufacture which may be applied to various uses. For example, it may be employed as the outer layer or layers 65 of a composite wall-board or siding, the body of the board consisting of suitable material such as an asphalt cement mixed with binding material, such as asbestos fiber, clay, sawdust, wood fiber, stone dust, sand, etc. When one side of the composite sheet is not 70 exposed to the weather (as, for instance, the bottom side of roofing), that side need not be waterproofed, or it may be waterproofed with asphalt or other suitable material, the color of which is not of consequence.

The composite sheet just described may be used in the manufacture of shingles, the sheet being formed of any suitable thickness, and made tapering, if desired.

In the accompanying drawing, Figure 1 75 is a cross-sectional view of a composite roofing or board embodying my invention. Fig. 2 is a face view of a sheet of asbestos paper waterproofed in accordance with my invention. Fig. 3 illustrates three different designs or arrangements of lines and colors 80 which may be imprinted upon the sheet.

1 denotes the sheets of asbestos paper and 2 an intermediate layer of suitable material such as that herein described.

When the word "rubber" is used in the 85 following claims it is to be understood as signifying not only india rubber but also rubber substitutes or rubberlike bodies.

I claim as my invention:

1. An improved building material comprising a waterproof sheet of asbestos paper

the fibers of which are bound together by an oxidized oil incorporated therein.

2. An improved building material comprising a sheet of asbestos paper waterproofed by saturation with a binder consisting of non-asphaltic oxidizable oil in a volatile solvent.

3. A sheet of asbestos paper waterproofed by saturation with a solution of an oxidizable oil and rubber.

4. An improved building material com-

prising a waterproof sheet of asbestos paper the fibers of which are bound together by an oxidized oil incorporated therein, said sheet having a hard waterproof surface, 15 provided with a design printed thereon.

In testimony whereof I affix my signature in the presence of two witnesses.

EDWARD J. SCHRODER.

Witnesses:

CHARLES W. HILLS, Jr.,  
GEORGE L. CHINDAHL.